

## UNITED STATES PATENT OFFICE

2,297,701

## PROCESS OF DYEING ANIMAL FIBERS

Gustave Theodore Hug, Penns Grove, N. J., assignor to E. I. du Pont de Nemours & Company, Wilmington, Del., a corporation of Delaware

No Drawing. Application April 11, 1940,  
Serial No. 329,108

5 Claims. (Cl. 8—36)

This invention relates to the dyeing of animal fibers with indigoid and anthraquinone types of vat colors and more particularly to the pretreatment of wool to increase its affinity for indigo and other vat dyes.

This invention has as an object the dyeing of woolen piece goods continuously with vat dyes. A further object is the dyeing of animal fibers in the form of piece goods, skeins or raw stock with indigoid and anthraquinone vat dyes. Other and further important objects of this invention will appear as the description proceeds.

These objects are accomplished by the following invention which consists of pretreating the woolen material by padding it through a solution or suspension of a sulfur-containing vat-reducing agent, for instance a compound selected from the group consisting of formamidine sulfonic acid, hydrosulfite, the aldehyde sulfoxylates, the bisulfites and the water-soluble sulfides, steaming the padded material, rinsing, and subsequently dyeing it in a bath containing a reduced indigoid or anthraquinone vat dye. These vat dyes may be reduced by any of the known methods but a caustic-soda-hydrosulfite reduction is preferred.

In place of padding and steaming, the pretreatment can be effected by immersing the wool in a bath containing one of the compounds mentioned above and treating at elevated temperatures as more fully explained below. Dyeings of indigoid and anthraquinone vat dyes on wool pretreated by either of these methods are considerably stronger than when the pretreatment is omitted. The concentration of the pretreating agent in the pad liquor is not critical; but the preferred range is about 2 to 3 ounces per gallon. Padding may be carried out at any temperature, although temperatures of 140 to 160° F. insure better penetration of the wool. After padding, the impregnated material is steamed at atmospheric pressure, preferably for 3 minutes, and rinsed.

In the alternative method mentioned above, the wool is treated in the form of piece goods, skeins or raw stock, in a bath containing 3 to 5%, based on the weight of the material, of one of the compounds mentioned above for 5 to 30 minutes at 160° to 212° F. The preferred method is a treatment for 15 minutes at 200° F. While temperatures below 160° F. may be employed, they cannot be considered commercially practical due to the proportionate increase in time necessary to obtain the desired effect.

After pretreating by either one of the described

methods, the material may be dyed in a reduced solution of a vat dye. Any normal procedure for the dyeing of wool is satisfactory, where precautions are taken to avoid excess alkalinity which has a deleterious effect on the wool.

Besides formamidine sulfonic acid, other suitable pretreating agents are sodium and zinc hydrosulfite, sodium, zinc and basic zinc formaldehyde sulfoxylate, sodium, potassium and zinc bisulfite, sodium and potassium sulfide. It will be clear from these examples, and numerous others which I have tried, that the agents suitable for this invention are compounds of the type generally employed as vat-reducing agents, but characterized further by containing sulfur in the molecule. However, it should not be inferred that these agents have the function of assisting merely in the reduction of the vat dye in the subsequent dyeing step, inasmuch as I have found that the impregnation agent may be, and in the preferred procedure usually is, rinsed completely out of the fiber prior to the dyeing step, without sacrificing the benefit of this treatment upon the strength of the dyeing obtained.

An advantage of this invention over conventional methods is that the affinity of wool for vat dyes is increased. This feature is of particular value for the continuous dyeing of woolen piece goods with vat colors, for example indigo. Thus, due to the increased affinity, it is possible by this invention to obtain deep navy shades on wool by dyeing for only 3 minutes in a bath containing 3 ounces per gallon of reduced indigo, 20% paste, whereas when using conventional methods, it would be necessary to dye for 10 minutes, then oxidize and dye for an additional 10 minutes in a second bath, to obtain a similar depth of shade. Such a procedure obviously would not lend itself to a continuous dyeing process.

A further advantage is the fact that the increased affinity of the wool permits the production of light to dark shades with vat colors in a much shorter period of time than when using conventional methods. This shorter dyeing time furthermore reduces the possible deleterious effect of alkalies, necessary for the reduction of vat dyes, on the wool fibers.

A further advantage is the fact that wool pretreated as described can be readily dyed with those vat colors which normally have little or no affinity for wool, for example "Ponsol" Blue GD Double Paste (Color Index #1113).

Without limiting my invention to any particular procedure, the following examples are given

to illustrate my preferred mode of operation. Parts mentioned are by weight.

*Example 1*

Wool felt is padded at 150° F. through an aqueous solution containing 2½ ounces per gallon of formamidine sulfonic acid. The time of immersion is approximately 3 seconds (operative range 1 to 10 seconds) and the squeezing rolls are adjusted to permit the material to retain 100% of its weight of moisture. The impregnated material is then run directly into a steamer where it is steamed for 3 minutes (operative range 1 to 5 minutes) at atmospheric pressure and then run through a rinse box containing water of about 80° F. After squeezing to remove excess moisture the steamed and rinsed felt is run through a vat containing 3 ounces per gallon of reduced indigo, 20% paste. The indigo is first reduced according to normal procedure with hydrosulfite and caustic soda, and the bath is rendered alkaline with ammonia. Time of immersion in the indigo vat is 3 minutes at 125° F. After dyeing, the material is squeezed to remove excess moisture and oxidized by skying or by chemical means.

The dyeings so obtained are at least 50% stronger in shade than if untreated wool is dyed in an indigo vat of the same strength.

*Example 2*

Wool crepe is pretreated by padding through a solution containing 2½ ounces per gallon of sodium formaldehyde sulfoxylate, steaming and rinsing as described in Example 1. After dyeing with indigo 20% paste as described in Example 1, much heavier shades are obtained than if the pretreatment is omitted.

*Example 3*

Wool flannel is pretreated by padding through a solution containing 2 ounces per gallon of sodium bisulfite, steaming and rinsing, and subsequently dyeing with indigo 20% paste as described in Example 1. Much heavier shades are obtained than when the pretreatment is omitted.

*Example 4*

Wool skeins are pretreated by immersing for 15 minutes at 200° F., at a volume of 40:1, in a bath containing 5% formamidine sulfonic acid, based on the weight of the material. After draining and rinsing, the skeins are dyed for 10 minutes in a bath containing one ounce per gallon of reduced indigo 20% paste. After oxidizing, the pretreated skeins are much heavier in shade than material not thus pretreated.

Equally satisfactory results are obtained by the substitution of 5% sodium sulfide, based on the weight of the material, for the formamidine sulfonic acid.

*Example 5*

Wool crepe is pretreated by padding through a solution containing 2½ ounces per gallon of formamidine sulfonic acid, steaming and rinsing as described in Example 1. It is then passed through a bath, for 2 minutes at 125° F., containing one ounce per gallon of reduced "Ponsol" Red BN Double Paste (Color Index #1162). The vat dye was reduced with hydrosulfite and caustic soda, as commonly employed in the dyeing of cotton. To present an undue deleterious action of the alkali on the wool, however, only ½% of the normal amount of caustic soda was used for reduction. After passage through the dye bath, the wool crepe is squeezed to remove excess moisture.

and oxidized by chemical means. Dyeings on pretreated material are at least 50% stronger than dyeings on untreated crepe.

*Example 6*

5 Wool crepe is pretreated with formamidine sulfonic acid as described in Example 1. After steaming and rinsing the material is dyed as described in Example 5, the color selected in this case being "Ponsol" Jade Green Double Paste (Color Index #1101). The dyeing is considerably stronger than that obtainable on untreated wool.

*Example 7*

15 Wool crepe is pretreated with formamidine sulfonic acid as described in Example 1, and dyed as described in Example 5, the color selected being "Sulfanethrene" Blue 2BD Paste (Color Index #1184). Pretreated material is dyed very much 20 heavier than untreated wool.

*Example 8*

Wool crepe is pretreated with formamidine sulfonic acid as described in Example 1 and dyed as described in Example 5, the color selected being 25 "Ponsol" Blue GD Double Paste (Color Index #1113). The dyeing is very much stronger than that obtainable on untreated material.

*Example 9*

30 Wool crepe is pretreated with formamidine sulfonic acid as described in Example 1 and dyed as described in Example 5, the color selected being "Ponsol" Violet AR Paste (Color Index #1135). The dyeing is very much stronger than that obtainable on untreated material.

*Example 10*

Wool crepe is pretreated with sodium formaldehyde sulfoxylate as described in Example 2 and dyed as described in Example 5, the color selected in this case being "Ponsol" Blue Green FFB Double Paste (Color Index #1173). The dyeing is very much stronger than if the pretreatment is omitted.

*Example 11*

55 Wool crepe is pretreated with sodium formaldehyde sulfoxylate as described in Example 2 and dyed as described in Example 5, the color selected in this case being "Ponsol" Golden Orange RRT Paste (Color Index #1097). The dyeing is very much stronger than is obtainable on untreated material.

*Example 12*

60 Wool crepe is pretreated with formamidine sulfonic acid as described in Example 1. After steaming and rinsing, the material is padded at 140° F. through a solution containing 2 ounces per gallon of the leuco ester of "Ponsol" Jade Green (Color Index #1101) and one ounce per gallon sodium nitrite. The padded material is then developed at 70 to 80° F. for 3 minutes in a 2% solution of sulfuric acid, rinsed and soaped. 65 Much heavier dyeings are obtained on pretreated wool crepe than on untreated material.

Equally satisfactory results are obtainable if the leuco ester of the vat dye is applied by dyeing in a beek or jig instead of by padding.

70 It will be understood that my invention is susceptible of wide variation in details, within the skill of those versed with this art, without departing from the spirit of this invention.

I claim:

1. In a process of dyeing wool fiber with vat

dyestuffs, the improvement which comprises first treating the fiber in an aqueous bath containing a sulfur-containing vat-reducing agent but no added alkali and no vat color, the concentration of the agent in the bath being insufficient to reduce the wool to a rubber-like condition; heating the impregnated fiber, and then subjecting the same to vat dyeing in a bath containing the chosen vat color, alkaline agents and reducing agents.

2. A process as in claim 1, the heating being effected simultaneously with the impregnation, by using a hot impregnation bath, at a temperature between 160° and 212° F.

3. A process as in claim 1, the heating being effected by subjecting the fiber to steam ageing at atmospheric pressure, subsequent to treatment with the impregnation bath.

4. A process of dyeing wool fiber, which comprises pretreating the same in an aqueous bath containing a sulfur-containing vat-reducing agent in quantity not exceeding 3 ounces per gal-

lon, but no added alkali and no coloring matter, and heating the treated fiber; then rinsing the fiber and dyeing the same from an alkaline aqueous bath containing a reduced vat dye of the group consisting of anthraquinone vat dyes and indigoid vat dyes, the time of dyeing not exceeding 3 minutes; and finally subjecting the dyed fiber to an oxidation treatment, to reoxidize the dye on the fiber.

10 5. A process for the continuous dyeing of wool with indigo, which consists in the impregnation of the wool with an aqueous solution of formamidine sulfonic acid at a concentration of from 2 to 3 ounces per gallon steaming the fiber and rinsing; the time of impregnation not exceeding 10 seconds, and the time of steaming not exceeding 5 minutes, then immersing the wool in an aqueous alkaline bath containing reduced indigo, removing the fiber from the bath and oxidizing the 20 color on the fiber.

GUSTAVE THEODORE HUG.